



US005306465A

**United States Patent [19]**

Caron et al.

[11] **Patent Number:** 5,306,465[45] **Date of Patent:** Apr. 26, 1994

[54] **COPPER ALLOY HAVING HIGH STRENGTH AND HIGH ELECTRICAL CONDUCTIVITY**

[75] Inventors: Ronald N. Caron, Branford; John F. Breedis, Trumbull, both of Conn.

[73] Assignee: Olin Corporation, New Haven, Conn.

[21] Appl. No.: 971,499

[22] Filed: Nov. 4, 1992

[51] Int. Cl.<sup>5</sup> ..... C22C 9/00

[52] U.S. Cl. ..... 420/492; 148/432

[58] Field of Search ..... 420/492; 148/432

[56] **References Cited**

**U.S. PATENT DOCUMENTS**

2,025,662 12/1936 Hensel .  
 2,479,311 8/1949 Christensen et al. .  
 3,194,655 7/1965 Pels et al. .  
 3,392,016 7/1968 Opie et al. .  
 3,928,028 12/1975 Yarwood .  
 4,047,980 9/1977 Watson et al. .  
 4,224,066 9/1980 Watson et al. .  
 4,049,426 9/1977 Watson et al. .  
 4,589,930 5/1986 Kumagal .  
 4,594,221 6/1986 Caron et al. .  
 4,631,237 12/1986 Dommer et al. .  
 4,749,548 6/1988 Akutsu et al. .  
 4,872,048 10/1989 Akutsu et al. ..... 356/67  
 5,004,520 4/1991 Tsuji et al. .  
 5,017,250 5/1991 Ashok .

**FOREIGN PATENT DOCUMENTS**

80104479 2/1981 European Pat. Off. .  
 59-193233 11/1984 Japan ..... 422/492

1157163 7/1969 United Kingdom .  
 1353430 5/1974 United Kingdom .  
 1373049 11/1974 United Kingdom .  
 1414289 11/1975 United Kingdom .  
 1525355 9/1978 United Kingdom .  
 1549107 7/1979 United Kingdom .  
 1566776 5/1980 United Kingdom .  
 2070057A 9/1981 United Kingdom .  
 2259836A 6/1985 United Kingdom .

**OTHER PUBLICATIONS**

Metals Handbook, Tenth Edition, vol. 2 (1990), pp. 259-263, 266, 281 and 290-291.

Pareige et al. "Precipitation in Dilute Cu Fe Ti Alloy: an Atom-Probe Study" appearing in Memoires Et Etudes Scientifiques Revue De Metallurgie, vol. 89, No. 5, May 1992 at pp. 311-316.

Yamaguchi et al, "31 Copper-Iron-Titanium Precipitation Hardenable Dilute Alloys for Terminal and Connector Applications" appearing in Copper '90, Refining, Fabrication, Markets, Oct. 1990 at pp. 517-525.

*Primary Examiner*—Deborah Yee  
*Attorney, Agent, or Firm*—Gregory S. Rosenblatt

[57] **ABSTRACT**

There is disclosed a copper base alloy which contains specified additions of chromium, zirconium, cobalt and/or iron, and titanium as well as methods for the processing of the copper alloy. One method of processing results in a copper alloy having high strength and high electrical conductivity. A second method of processing results in a copper alloy with even higher strength and a minimal reduction in electrical conductivity.

**11 Claims, 2 Drawing Sheets**





FIG.2



FIG.1



FIG.3

## COPPER ALLOY HAVING HIGH STRENGTH AND HIGH ELECTRICAL CONDUCTIVITY

### FIELD OF THE INVENTION

This invention relates to copper alloys having high strength and high electrical conductivity. More particularly, a copper-zirconium-chromium base alloy is modified by additions of cobalt (and/or iron) and titanium to form a copper alloy for electrical and electronic applications.

### BACKGROUND OF THE INVENTION

Electrical components such as connectors and electronic components such as leadframes are manufactured from copper alloys to exploit the high electrical conductivity of copper. Pure copper such as C10200 (oxygen-free copper having a minimum copper content by weight of 99.95%) has a yield strength in a spring temper of about 37 kg/mm<sup>2</sup> (52 ksi) which is too weak for applications in which the component is subject to forces associated with insertion and removal. To increase the strength of copper, a wide array of alloying elements have been added to copper. In most cases, there is a tradeoff between the increase in yield strength achieved by the alloying addition with a resultant decrease in the electrical conductivity.

Throughout this application, alloy designations such as C10200 utilize the Unified Numbering System designations. Compositional percentages are in weight percent unless otherwise noted.

For electrical and electronic applications zirconium and mixtures of zirconium and chromium are frequently added to copper. For example, copper alloy C15100 (nominal composition 0.05–0.15% zirconium and the balance copper) has an electrical conductivity of 95% IACS (IACS stands for International Annealed Copper Standard where pure copper has an electrical conductivity of 100%). C15100 has a spring temper yield strength of no more than 46 kg/mm<sup>2</sup> (66 ksi). A copper-zirconium intermetallic phase precipitates from the copper matrix as a discrete second phase following heat treatment (precipitation hardening) increasing the strength of the alloy. However, the yield strength of C15100 is still too low for the current trend to higher strength connectors and leadframes in miniaturized applications.

Higher strength is obtained by adding a mixture of chromium and zirconium to copper. C18100 (nominal composition 0.4%–1.0% chromium, 0.08%–0.2% zirconium, 0.03%–0.06% magnesium and the balance copper) has an electrical conductivity of 80% IACS at a yield strength of from 47–50 kg/mm<sup>2</sup> (67 to 72 ksi). The electrical conductivity of C18100 is acceptable, however, the yield strength is slightly lower than desired. Also, a chromium content above the maximum solid solubility of chromium in copper, about 0.65%, leads to large second phase dispersions which contribute to a poor surface quality and non-uniform chemical etching characteristics.

For leadframes requiring high heat dissipation to prolong semiconductor device life and electrical connectors carrying high currents where ohmic heating is detrimental, it is desirable to have an electrical conductivity above about 70% IACS and a yield strength above about 56 kg/mm<sup>2</sup> (80 ksi).

The alloy should have good stress relaxation resistance properties both at room temperature and at ele-

vated (up to 200° C.) service temperatures. When an external stress is applied to a metallic strip, the metal reacts by developing an equal and opposite internal stress. If the metal is held in a strained position, the internal stress will decrease as a function of both time and temperature. This phenomenon, called stress relaxation, occurs because of the replacement of elastic strain in the metal to plastic, or permanent strain, by microplastic flow. Copper based electrical connectors are frequently formed into spring contact members which must maintain above a threshold contact force on a mating member for prolonged times. Stress relaxation reduces the contact force to below the threshold leading to an open circuit. Copper alloys for electrical and electronic applications should, therefore, have high resistance to stress relaxation at both room and high ambient temperatures.

The minimum bend radius (MBR) determines how tight a bend may be formed in a metallic strip without "orange peeling" or fracture along the outside radius of the bend. The MBR is an important property of leadframes where the outer leads are bent at a 90° angle for insertion into a printed circuit board. Connectors are also formed with bends at various angles. Bend formability, MBR/t where t is the thickness of the metal strip, is the ratio of the minimum radius of curvature of a mandrel around which the metallic strip can be bent without failure and the thickness of the metal.

$$\frac{MBR}{t} = \frac{\text{Radius of Curvature of Mandrel}}{\text{Thickness of Metal}} \quad (1)$$

An MBR/t of under about 2.5 is desired for bends made in the "good way", bend axis perpendicular to the rolling direction of the metallic strip. An MBR of under about 2.5 is desired for bends made in the "bad way", bend axis parallel to the rolling direction of the metallic strip.

In summary a desirable copper alloy for electrical and electronic applications would have all of the following properties:

Electrical conductivity equals greater than 70% IACS.

Yield strength greater than 56 kg/mm<sup>2</sup> (80 ksi).

Resistance to stress relaxation.

MBR/t less than 2.5 in the "good way" and "bad way".

The copper alloy should resist oxidation and etch uniformly. The uniform etch leads to sharp and smooth vertical lead walls on etched leadframes. A uniform chemical etch during precleaning also promotes good coatings by electrolytic or electroless means.

U.S. Pat. No. 4,872,048 to Akutsu et al. discloses copper alloys for leadframes. The patent discloses copper alloys containing 0.05–1% chromium, 0.005–0.3% zirconium and either 0.001–0.05% lithium or 5–60 ppm carbon. Up to about 2% of various other additions may also be present. Two disclosed examples are Alloy 21 (0.98% chromium, 0.049% zirconium, 0.026% lithium, 0.41% nickel, 0.48% tin, 0.63% titanium, 0.03% silicon, 0.13% phosphorous, balance copper) with a tensile strength of 80 kg/mm<sup>2</sup> (114 ksi) and an electrical conductivity of 69% IACS and Alloy 75 (0.75% chromium, 0.019% zirconium, 30 ppm carbon, 0.19% cobalt, 0.22% tin, 0.69% titanium, 0.13% niobium, balance

copper) with a tensile strength of 73 kg/mm<sup>2</sup> (104 ksi) and an electrical conductivity of 63% IACS.

Great Britain Patent Specification No. 1,353,430 to Gosudarstvenny Metallov, discloses copper-chromium-zirconium alloys containing tin and titanium. Alloy 1 contains 0.5% chromium, 0.13% titanium, 0.25% tin, 0.12% zirconium, balance copper with a tensile strength of 62-67 kg/mm<sup>2</sup> (88-95 ksi) and an electrical conductivity of 72% IACS.

Great Britain Patent Specification No. 1,549,107 to Olin Corporation, discloses copper-chromium-zirconium alloys containing niobium. Dependent on the method of processing, an alloy containing 0.55% chromium, 0.15% zirconium, 0.25% niobium and the balance copper has a yield stress of from 51-64 kg/mm<sup>2</sup> (73-92 ksi) and an electrical conductivity of 71-83% IACS.

#### SUMMARY OF THE INVENTION

It is apparent that there remains a need in the art for a copper alloy which satisfies the requirements specified above. Accordingly, it is an object of the present invention to provide such an alloy. It is a feature of the invention that the copper alloy is a copper-chromium-zirconium alloy containing specific concentrations of cobalt and titanium; iron and titanium; or cobalt, iron and titanium. Another feature of the invention is that the atomic percent ratio of cobalt to titanium; iron to titanium; or cobalt plus iron to titanium is controlled to provide high conductivity while retaining the strength of the alloy.

It is an advantage of the present invention that the claimed copper alloys have a yield strength above about 56 kg/mm<sup>2</sup> (79 ksi) and with the addition of multiple in process aging anneals, the yield strength is increased to above about 62 kg/mm<sup>2</sup> (89 ksi). Still another advantage of the invention is that the electrical conductivity of the claimed alloys is above 73% IACS and in some embodiments exceeds 77% IACS. It is a further advantage of the invention that the copper alloys exhibit excellent strength relaxation resistance with over 95% of the stress remaining after exposure to 150° C. for 3,000 hours. Yet a further advantage of the invention is that following some processing embodiments, the MBR/t of the alloy is about 1.8 in the good way and about 2.3 in the bad way for the claimed copper alloys.

Accordingly, there is provided a copper alloy consisting essentially of from an effective amount up to 0.5% by weight chromium; from about 0.05 to about 0.25% by weight zirconium; from about 0.1 to about 1% by weight of M, where M is selected from the group consisting of cobalt, iron and mixtures thereof; from about 0.05% to about 0.5% by weight titanium; and the balance copper.

The above stated objects, features and advantages will become more apparent from the specification and drawings which follows.

#### BRIEF DESCRIPTION OF THE DRAWINGS

FIG. 1 shows in block diagram the initial processing of a copper alloy containing chromium, zirconium, cobalt and/or iron and titanium in accordance with the invention.

FIG. 2 shows in block diagram a first embodiment to further process the copper alloy for high strength and high electrical conductivity.

FIG. 3 shows in block diagram a second embodiment to further process the copper alloy with extra high strength with a minimal loss of electrical conductivity.

#### DETAILED DESCRIPTION OF THE PREFERRED EMBODIMENTS

The copper alloys of the invention consist essentially of chromium, zirconium, cobalt and/or iron and titanium. The chromium is present in an amount of from that effective to increase strength through precipitation hardening to about 0.5%. Zirconium is present in an amount from about 0.05% to about 0.25%. Cobalt is present in an amount from about 0.1% to about 1%. Either a portion or all of the cobalt may be substituted with an equal weight percent of iron. Titanium is present in an amount of from about 0.05% to about 0.5%. The balance of the alloy is copper.

Chromium—Chromium is present in the alloy in an amount from that effective to increase the strength of the alloy through precipitation hardening (aging) up to about 0.5%. If the chromium content is above about 0.5%, the maximum solid solubility limit of chromium in copper is approached and a coarse second phase precipitate develops. The coarse precipitate detrimentally affects both the surface quality and the etching and plating characteristics of the copper alloy without increasing the strength of the alloy. The cobalt, iron and titanium also present in the alloy combine to form Co<sub>2</sub>Ti or Fe<sub>2</sub>Ti. If excess iron, cobalt or titanium remains unreacted and in solid solution in the copper matrix, electrical conductivity is decreased. The chromium ties up residual iron, cobalt or titanium to reduce this decrease in electrical conductivity. A preferred chromium content is from about 0.1% to about 0.4% and a most preferred chromium content is from about 0.25% to about 0.35%.

Zirconium—The zirconium content is from about 0.05% to about 0.25%. If the zirconium content is too low, the alloy has poor resistance to stress relaxation. If the zirconium content is too high, coarse particles form which detrimentally affect both the surface quality and the etching characteristics of the alloy without providing any increase in strength. A preferred zirconium content is from about 0.1% to about 0.2%.

Transition Element ("M")—A transition Element ("M") selected from the group consisting of cobalt, iron and mixtures thereof, is present in an amount of from about 0.1% to about 1%. While the cobalt and iron are generally interchangeable, iron provides a slight increase in strength (about a 4-5 ksi improvement) with a slight reduction in electrical conductivity (about a 5-6% IACS decrease). If the cobalt and/or iron content is too high, a coarse second phase particle forms during casting. The coarse precipitate detrimentally affects both the surface quality and the etching characteristics of the alloy. If there is insufficient titanium or chromium such that "M" remains in solid solution in the copper matrix, the electrical conductivity of the alloy is decreased. If the cobalt and/or iron content is too low, the alloy does not undergo precipitation hardening through aging and there is no corresponding increase in the strength of the alloy. A preferred amount of cobalt and/or iron is from about 0.25% to about 0.6%. The most preferred amount is from about 0.3% to about 0.5%.

Other transition elements which are reactive with titanium may be used. Applicants believe that some or

all of the cobalt and/or iron may be replaced with nickel.

Less reactive transition metals such as manganese are not preferred. Residual manganese and titanium in solid solution reduce electrical conductivity to unacceptable levels.

Titanium—Titanium is present in an amount of from about 0.05% to about 0.5%. Titanium combines with "M" to form a second phase precipitate  $\text{Co}_2\text{Ti}$  or  $\text{Fe}_2\text{Ti}$ . The preferred ratio of cobalt and/or iron to titanium is (in atomic percent) about 2:1. While it is believed that any ratio in the range of from about (in atomic percent) 1.5:1 to about 3:1 is effective, the preferred ratio of cobalt and/or iron to titanium is (in atomic percent) 2:1. As the content of the cobalt, iron and titanium vary from this ratio, the excess remains in solid solution in the copper matrix, reducing the electrical conductivity of the alloy

The alloys of the invention are formed by any suitable process. Two preferred methods are illustrated in FIGS. 1-3. FIG. 1 illustrates in block diagram the process steps generic to both preferred methods. FIG. 2 illustrates subsequent processing steps to produce an alloy having both high strength and high electrical conductivity. FIG. 3 illustrates in block diagram alternative processing steps to produce an alloy having even higher strength, with a minimal sacrifice in electrical conductivity.

With reference to FIG. 1, the alloys are cast 10 by any suitable process. In one exemplary process, cathode copper is melted in a silica crucible under a protective charcoal cover. The desired amount of cobalt and/or iron is then added. Titanium is added next to the melt, followed by zirconium. The melt is then poured into a steel mold and cast into an ingot.

The ingots are homogenized 12 by heating to a temperature generally between about 850° C. and 1050° C. for from about 30 minutes to about 24 hours. Preferably, homogenization is about 900° C.-950° C. for about 2-3 hours.

Alternatively, the ingot is cast directly into a thin slab, known in the art as "strip casting". The slab has a thickness of from about 2.5 mm to about 25 mm (0.1-1 inch). The cast strip is then either cold rolled or treated by a post casting recrystallization/homogenization anneal and then cold rolled.

Following homogenization 12, the ingot is hot rolled 14 to a reduction in excess of about 50% and preferably to a reduction on the order of from about 75% to about 95%. Throughout this application, reductions by rolling are given as reductions in cross sectional area unless otherwise specified. The hot roll reduction 14 may be in a single pass or require multiple passes. Immediately following the last hot roll reduction 14, the ingot is rapidly cooled to below the aging temperature, typically by quenching 16 in water to room temperature to retain the alloying elements in solid solution. Each of the quench steps specified in Applicants' processes are preferred, but optional, each quench step may be replaced with any other means of rapid cooling known in the art.

Following quenching 16, two different sequences of processing steps result in alloys with slightly different properties. A first process (designated "Process 1") is illustrated in FIG. 2. The alloy achieves high strength and high electrical conductivity. A second process (designated "Process 2") achieves higher strength with a minimal sacrifice of electrical conductivity.

FIG. 2 illustrates Process 1. The alloy is cold rolled 18 to a reduction in excess of about 25% and preferably to a reduction of from about 60% to about 90%. The cold roll 18 may be a single pass or multiple passes with or without intermediate recrystallization anneals. Following the cold roll 18, the alloy is solutionized 20 by heating to a temperature from about 750° C. to about 1050° C. for from about 30 seconds to about 2 hours. Preferably, the solutionization 20 is at a temperature of from about 900° C. to about 925° C. for from about 30 seconds to 2 minutes.

The alloy is next quenched 22 and then cold rolled 24 to final gauge. The cold roll 24 is a reduction in excess of about 25% and preferably in the range of from about 60% to about 90%. The cold roll 24 may be a single pass or in multiple passes with or without intermediate recrystallization anneals.

After the alloy is reduced to final gauge by cold roll 24, the alloy strength is increased by a precipitation aging 26. The alloy is aged by heating to a temperature of from about 350° C. to about 600° C. for from about 15 minutes to about 8 hours. Preferably, the alloy is heated to a temperature of from about 425° C. to about 525° C. for from about 1 to about 2 hours. Process 1 is utilized when the optimum combination of strength, electrical conductivity, and formability is required.

If higher strength is required, at a slight reduction in electrical conductivity, Process 2 as illustrated in FIG. 3 is utilized. Following the quench 16 (FIG. 1), the alloy is cold rolled 28 to solutionizing gauge. The cold roll reduction is in excess of about 25% and preferably in the range of from about 60 to about 90%. The cold roll step 28 may be a single pass or multiple passes with or without intermediate recrystallization anneals.

Following cold rolling 28, the alloy is solutionized 30 by heating to a temperature of from about 750° C. to about 1050° C. for from about 15 seconds to about 2 hours. More preferably, the solutionizing temperature is from about 900° C. to about 925° C. for from about 30 seconds to about 2 minutes. Following solutionizing 30, the alloy is rapidly cooled such as by quenching 32, typically in water, to below the aging temperature.

The alloy is then cold rolled 34 to a reduction of from about 25% to about 50%. The reduction may be a single pass or multiple passes with intermediate solutionizing recrystallization anneals. Following the cold roll 34, the alloy is age hardened 36 at temperatures sufficiently low to avoid recrystallization. The aging 36 is preferably at a temperature of from about 350° C. to about 600° C. for a time of from about 15 minutes to about 8 hours. More preferably, the non-recrystallizing precipitation hardening treatment 36 is at a temperature of from about 450° C. to about 500° C. for from about 2 to about 3 hours.

Following the non-recrystallizing aging 36, the alloy is cold rolled 38 to a reduction of from about 30% to about 60%. Following the cold roll step 38, the alloy is optionally given a second non-recrystallizing precipitation hardening anneal 40 at a temperature in the range of from about 350° C. to about 600° C. for from about 30 minutes to about 5 hours. Preferably, this optional second non-recrystallizing precipitation hardening anneal 40 is at a temperature of from about 450° C. to about 500° C. for from about 2 to 4 hours. The precise time and temperature for the second optional non-recrystallizing precipitation hardening step 40 is selected to maximize the electrical conductivity of the alloy.

The alloy is then cold rolled 42 by from about 35% to about 65% reduction to final gauge in single or multiple passes, with or without intermediate sub-recrystallization anneals. Following the cold roll 42, the alloy is given a stabilization relief anneal 44 at a temperature of 5 from about 300° C. to about 600° C. for from about 10 seconds to about 10 minutes for a strand anneal. For a bell anneal, the stabilization relief anneal 44 is at a temperature of up to about 400° C. for from about 15 minutes to about 8 hours. More preferred is a bell anneal at 10 about 250° C. to about 400° C. for from about 1 to about 2 hours. Following the stabilization anneal 44, the alloy is quenched 46 if strand annealed. A quench is generally not utilized following a bell anneal. Process 2 produces an alloy having maximum strength with a minimal sacrifice in electrical conductivity. 15

In another process embodiment, a homogenization anneal (reference numeral 48 in FIG. 1) is included with either Process 1 or Process 2. The homogenization anneal 48 is inserted between the hot roll step 14 and the 20 solutionizing step (20 in FIG. 2 or 30 in FIG. 3), before or after the cold roll step (18 in FIG. 2 or 28 in FIG. 3). The homogenization anneal 48 is at a temperature of 25 from about 350° C. to about 650° C. for from about 15 minutes to about 8 hours. Preferably, the homogenization anneal 48 is at a temperature of from about 550° C. to about 650° C. for from about 6 to about 8 hours. 30

Generally, the alloys of Process 1 are utilized where high strength, high electrical conductivity and formability are required such as in connector and leadframe 35 applications. Process 2 is utilized in applications where higher strength and excellent stress relaxation resistance are required and some minimal loss in electrical conductivity is tolerated, for example, electrical connectors subject to elevated temperature such as for automotive 30 applications as well as leadframes requiring high strength leads.

The advantages of the alloys of the invention will be apparent from the Examples which follow. The Examples are intended to be exemplary and not to limit the 40 scope of the invention.

### EXAMPLES

The electrical and mechanical properties of the alloys of the invention were compared with copper alloys 45 conventionally used in leadframe and connector applications. Table 1 lists the alloy compositions. The alloys preceded by an asterisk, H, I and P are alloys of the invention while other alloys are either conventional alloys or, as to alloys G, K and L, variations of preferred compositions to illustrate either the contribution of chromium or the ratio of "M" to titanium.

TABLE 1

| ALLOY | ZR   | ALLOY COMPOSITION |      |      |      | MG   | OTHER   |
|-------|------|-------------------|------|------|------|------|---------|
|       |      | CR                | CO   | FE   | TI   |      |         |
| A     | 0.13 | 0.80              | —    | —    | —    | 0.08 |         |
| B     | 0.20 | 0.32              | —    | —    | —    | 0.06 |         |
| C     | 0.25 | —                 | —    | —    | —    | —    |         |
| D     | 0.25 | 0.27              | 0.23 | —    | —    | —    |         |
| E     | 0.21 | 0.25              | —    | 0.32 | —    | —    |         |
| F     | 0.21 | 0.32              | —    | —    | 0.21 | —    |         |
| G     | 0.21 | —                 | —    | 0.43 | 0.23 | —    |         |
| *H    | 0.20 | 0.30              | 0.46 | —    | 0.24 | —    |         |
| *I    | 0.20 | 0.29              | —    | 0.43 | 0.23 | —    |         |
| J     | 0.20 | 0.26              | 0.25 | 0.27 | 0.22 | —    |         |
| K     | 0.20 | 0.35              | 0.28 | —    | 0.24 | —    |         |
| L     | 0.20 | 0.37              | —    | 0.24 | 0.24 | —    |         |
| M     | 0.19 | —                 | 0.66 | —    | 0.23 | —    |         |
| N     | —    | —                 | —    | 0.6  | —    | 0.05 | 0.18 P  |
| O     | —    | 0.3               | —    | —    | 0.1  | —    | 0.02 SI |
| *P    | 0.20 | 0.3               | 0.5  | —    | 0.2  | —    |         |
| Q     | 0.10 | —                 | —    | —    | —    | —    |         |
| R     | 0.25 | 0.27              | 0.23 | —    | —    | —    |         |

Alloys A through M and P were produced by the method described above. A 5.2 kg (10 pound) ingot of each alloy was made by melting cathode copper in a silica crucible under a protective charcoal cover, charging the required cobalt and/or iron additions, then adding the titanium addition followed by zirconium and magnesium. Each melt was then poured into a steel mold which upon solidification produced an ingot having a thickness of 4.45 cm (1.75 inches) and a length and width both 10.16 cm (4 inches). Alloys N and O are commercial alloys acquired as strip having an H08 (spring) temper. Alloy Q is alloy C15100 acquired as strip in a HR04 (hard relief anneal) temper.

Table 2 shows the electrical and mechanical properties of alloys A through M and R processed by Process 1. Alloys H, I and J have a higher strength than base line copper zirconium alloys (alloy C) as well as base line copper chromium zirconium alloys (alloy B). Surprisingly, alloys H, I and J which have about 0.30 weight percent chromium have a yield strength and ultimate tensile strength about equal to alloy A which has a chromium content almost three times as high.

The effect of chromium on enhancing conductivity is illustrated by comparing alloy G and alloy I. The only significant difference in composition between the alloys is the presence in alloy I of 0.29% chromium. The electrical conductivity of alloy I, 72.0% IACS, is significantly higher than the conductivity of alloy G 65.1% IACS.

The criticality of the atomic weight ratio of 2:1 for the (cobalt and/or iron):titanium is demonstrated by comparing alloys H and I which have the ratio of 2:1 to alloys K and L which have a ratio of about 1:1. While the strengths of alloys H and I and alloys K and L are 55 approximately equal, the electrical conductivity of alloys K and L are about 20% IACS lower.

TABLE 2

| ALLOY | CONDUCTIVITY<br>% IACS | PROPERTIES OF ALLOYS PROCESSED ACCORDING TO PROCESS 1 |     |                                 |     |                       |                  |
|-------|------------------------|-------------------------------------------------------|-----|---------------------------------|-----|-----------------------|------------------|
|       |                        | YIELD<br>STRENGTH                                     |     | ULTIMATE<br>TENSILE<br>STRENGTH |     | ELONGATION<br>PERCENT | MBR/T<br>(GW/BW) |
|       |                        | KG/MM <sup>2</sup>                                    | KSI | KG/MM <sup>2</sup>              | KSI |                       |                  |
| A     | 79.0                   | 56.7                                                  | 81  | 58.8                            | 84  | 9                     | 1.7/1.7          |
| B     | 77.6                   | 52.5                                                  | 75  | 55.3                            | 79  | 8                     | 1.4/2.3          |
| C     | 91.3                   | 44.1                                                  | 63  | 46.9                            | 67  | 8                     | 1.4/1.8          |
| D     | 74.7                   | 54.6                                                  | 78  | 56.0                            | 80  | 8                     | 1.4/1.8          |
| E     | 62.7                   | 52.5                                                  | 75  | 54.6                            | 78  | 9                     | 2.3/3.1          |
| F     | 36.0                   | 57.4                                                  | 82  | 60.2                            | 86  | 9                     | 1.8/3.1          |
| G     | 65.1                   | 57.4                                                  | 82  | 60.9                            | 87  | 10                    | 1.8/2.3          |

TABLE 2-continued

## PROPERTIES OF ALLOYS PROCESSED ACCORDING TO PROCESS 1

| ALLOY | CONDUCTIVITY<br>% IACS | YIELD<br>STRENGTH  |     | ULTIMATE<br>TENSILE<br>STRENGTH |     | ELONGATION<br>PERCENT | MBR/T<br>(GW/BW) |
|-------|------------------------|--------------------|-----|---------------------------------|-----|-----------------------|------------------|
|       |                        | KG/MM <sup>2</sup> | KSI | KG/MM <sup>2</sup>              | KSI |                       |                  |
| *H    | 77.5                   | 57.4               | 82  | 60.2                            | 86  | 8                     | 1.8/2.3          |
| *I    | 72.0                   | 58.1               | 83  | 60.9                            | 87  | 9                     | 1.8/2.3          |
| J     | 73.3                   | 55.3               | 79  | 59.5                            | 85  | 9                     | 1.5/1.8          |
| K     | 52.4                   | 58.8               | 84  | 60.9                            | 87  | 9                     | 2.3/2.3          |
| L     | 56.6                   | 62.3               | 89  | 64.4                            | 92  | 10                    | 2.3/2.3          |
| M     | 70.7                   | 49.0               | 70  | 51.1                            | 73  | 8                     | 1.8/2.3          |
| R     | 82.0                   | 51.1               | 73  | 53.2                            | 76  | 9                     | 1.4/1.8          |

Alloys D and R illustrates that for certain applications, the titanium may be eliminated. The copper-chromium-zirconium-cobalt alloys have strengths equal to alloys containing significantly higher chromium with better formability, etching and plating characteristics. The electrical conductivity is higher than that of titanium containing alloys but at a loss of strength. It is believed that the chromium, zirconium and cobalt ranges would be the same as that of the other alloys of the invention.

strength, is accompanying by almost no drop in electrical conductivity.

Process 2 results in alloys of the invention with an about 21 kg/mm<sup>2</sup> (30 ksi) yield strength improvement over binary copper zirconium alloys such as alloy C. The benefit of the chromium addition is apparent by comparing the electrical conductivity of alloy G (0% Cr) with that for alloy I (0.29% Cr). Alloy G has a conductivity of 59.3% IACS alloy I has a conductivity of 75.5% IACS.

TABLE 3

## PROPERTIES OF ALLOYS PROCESSED ACCORDING TO PROCESS 2

| ALLOY | CONDUCTIVITY<br>% IACS | YIELD<br>STRENGTH  |     | ULTIMATE<br>TENSILE<br>STRENGTH |     | ELONGATION<br>PERCENT | (GW/BW)<br>MBR/T |
|-------|------------------------|--------------------|-----|---------------------------------|-----|-----------------------|------------------|
|       |                        | KG/MM <sup>2</sup> | KSI | KG/MM <sup>2</sup>              | KSI |                       |                  |
| A     | 81.0                   | 56.7               | 81  | 57.4                            | 82  | 7                     | 2.2/2.4          |
| B     | 82.8                   | 50.4               | 72  | 51.8                            | 74  | 4                     | 2.1/2.9          |
| C     | 94.4                   | 43.4               | 62  | 44.8                            | 64  | 3                     | 1.9/3.1          |
| D     | 80.5                   | 54.6               | 78  | 56.0                            | 80  | 4                     | 2.4/3.8          |
| E     | 70.6                   | 53.9               | 77  | 55.3                            | 79  | 3                     | 2.8/5.2          |
| G     | 59.3                   | 62.3               | 89  | 64.4                            | 92  | 3                     | 2.4/5.0          |
| *H    | 77.1                   | 65.1               | 93  | 68.6                            | 98  | 3                     | 2.8/5.2          |
| *I    | 75.5                   | 64.4               | 92  | 65.8                            | 94  | 5                     | 3.0/5.2          |
| J     | 73.7                   | 62.3               | 89  | 65.8                            | 94  | 5                     | 2.3/5.2          |
| R     | 80.5                   | 54.6               | 78  | 56.0                            | 80  | 4                     | 2.4/3.8          |

Table 3 illustrates the properties of alloys A through E, G through J and R when processed by Process 2. The one exception is alloy C which was processed with a single in process aging anneal. Alloy C was cold rolled to 2.54 mm (0.10 inch) gauge from milled hot rolled plate (16 of FIG. 1) solutionized at 900° C. for 30 seconds and then water quenched. The alloy was then cold rolled to a 50% reduction, aged at 450° C. for 7 hours and then cold rolled with a 50% reduction to a 50 final gauge of 0.64 mm (0.025 inch). Alloy C was then relief annealed at 350° C. for 5 minutes.

The alloys of the invention, H, I and J, all have higher strength than the conventional alloys, including commercial alloy C181 (alloy A) which has a chromium content almost three times that of the alloys of the invention. In addition, the significant increase in strength, an increase of 5.6-8.4 kg/mm<sup>2</sup> (8-12 ksi) for the yield

TABLE 4

## STRESS RELAXATION - 150° C. EXPOSURE

| ALLOY | METHOD | PROCESS | YIELD<br>STRENGTH  |     | PERCENT STRESS<br>REMAINING<br>AFTER<br>3000 HOURS |
|-------|--------|---------|--------------------|-----|----------------------------------------------------|
|       |        |         | KG/MM <sup>2</sup> | KSI |                                                    |
| A     | AGED   | 56.7    | 81                 | 92  |                                                    |
| A     | 2-IPA  | 56.7    | 81                 | 87  |                                                    |
| C     | AGED   | 44.1    | 63                 | 89  |                                                    |
| C     | 1-IPA  | 43.4    | 62                 | 84  |                                                    |
| D     | AGED   | 54.6    | 78                 | 92  |                                                    |
| E     | AGED   | 52.5    | 75                 | 96  |                                                    |
| *H    | AGED   | 57.4    | 82                 | 95  |                                                    |
| *H    | 2-IPA  | 65.1    | 93                 | 85  |                                                    |
| *I    | AGED   | 58.1    | 83                 | 96  |                                                    |
| *I    | 2-IPA  | 58.1    | 83                 | 96  |                                                    |
| J     | 2-IPA  | 63.0    | 90                 | 96  |                                                    |
| Q     | HD/RA  | 39.2    | 56                 | 80  |                                                    |

TABLE 5

## COMPARISON OF LEADFRAME ALLOYS

| ALLOY | CONDUCTIVITY<br>% IACS | YIELD<br>STRENGTH  |     | MBR/T<br>GW/BW | 10 YEARS | 3000 HOURS | % STRESS<br>REMAINING<br>125° C. - |
|-------|------------------------|--------------------|-----|----------------|----------|------------|------------------------------------|
|       |                        | KG/MM <sup>2</sup> | KSI |                |          |            |                                    |
| N     | 77                     | 49                 | 70  | 2.0/2.5        | 78       | 75         |                                    |
| O     | 75                     | 49                 | 70  | 1.5/2.5        | 82       | 84         |                                    |

TABLE 5-continued

| COMPARISON OF LEADFRAME ALLOYS |                        |                    |     |                |                                                |
|--------------------------------|------------------------|--------------------|-----|----------------|------------------------------------------------|
| ALLOY                          | CONDUCTIVITY<br>% IACS | YIELD<br>STRENGTH  |     | MBR/T<br>GW/BW | % STRESS<br>REMAINING<br>105° C. -<br>10 YEARS |
|                                |                        | KG/MM <sup>2</sup> | KSI |                |                                                |
| *P                             | 75                     | 57.4               | 82  | 1.8/2.3        | 95                                             |
|                                |                        |                    |     |                | 92                                             |

Table 4 shows the stress relaxation of the alloys of the invention is better than that of either binary copper-zirconium alloys (alloys C and Q) or ternary copper-zirconium-chromium alloys (alloy A). In the second column of Table 4, "process type":

Aged=processing according to Process 1.

2-IPA=processing according to Process 2, with 2 In Process Anneals.

1-IPA=processing according to Process 2 with the second precipitation hardening anneal (40 in FIG. 3) deleted, 1 In Process Anneal.

One application for which the alloys of the invention are particularly suited is a leadframe for an electronic package. Alloys N and O represent alloys conventionally used in electronic packaging applications. Alloy N is copper alloy Cl97 and alloy O is one commercially available leadframe alloy. The alloy of the invention, alloy P, has a conductivity equivalent to those of the conventional leadframe alloys. The alloy P yield strength is considerably higher than that of alloys N and O. The minimum bend radius is less for alloy P and the resistance to stress relaxation is significantly improved.

While the alloys of the invention have particular utility for electrical and electronic applications such as electrical connectors and leadframes, the alloys may be used for any application in which high strength and/or good electrical conductivity is required. Such applications include conductive rods, wires and buss bars. Other applications include those requiring high electrical conductivity and resistance to stress relaxation such as welding electrodes.

The patents cited herein are intended to be incorporated by reference in their entireties.

It is apparent that there has been provided in accordance with this invention a copper alloy characterized by high strength and high electrical conductivity which is particularly suited for electric and electronic applications which fully satisfies the objects, means and advantages set forth hereinbefore. While the invention has been described in combination with specific embodiments and examples thereof, it is evident that may alternatives, modifications and variations will be apparent to those skilled in the art in light of the foregoing description. Accordingly, it intended to embrace all such alter-

natives, modifications and variations as fall within the spirit and broad scope of the appended claims.

We claim:

1. A copper alloy, consisting essentially of:  
an effective amount to increase strength up to about 0.5 weight percent chromium;  
from about 0.05 to about 0.25 weight percent zirconium;  
from about 0.1 to about 1.0 weight percent of "M"  
where "M" is selected from the group consisting of cobalt, iron, nickel and mixtures thereof; and  
from about 0.05 to about 0.5 weight percent titanium  
where the atomic ratio of "M" to titanium, M:Ti, is from about 1.5:1 to about 3.0:1.
2. The copper alloy of claim 1 wherein "M" is selected from the group consisting of cobalt, iron and mixtures thereof.
3. The copper alloy of claim 2 wherein the atomic ratio of "M" to titanium, M:Ti, is about 2:1.
4. The copper alloy of claim 2 wherein said chromium content is from about 0.1 to about 0.4 weight percent.
5. The copper alloy of claim 2 wherein said zirconium content is from about 0.1 to about 0.2 weight percent.
6. The copper alloy of claim 2 wherein said "M" content is from about 0.25 to about 0.6 weight percent.
7. A copper alloy, consisting essentially of;  
from about 0.1 to about 0.4 weight percent chromium;  
from about 0.1 to about 0.2 weight percent zirconium;  
from about 0.25 to about 0.6 weight percent of "M"  
where "M" is selected from the group consisting of cobalt, iron and mixtures thereof; and  
sufficient titanium such that the atomic ratio of "M" to titanium, M:Ti, is from about 1.5:1 to about 3.0:1.
8. The copper alloy of claim 7 wherein the atomic ratio of "M" to titanium, M:Ti, is about 2:1.
9. A leadframe manufactured from the alloy of claim 7.
10. An electrical connector manufactured from the alloy of claim 7.
11. A wire manufactured from the alloy of claim 7.

\* \* \* \* \*